



US008696103B2

(12) **United States Patent**  
Tsuji et al.

(10) Patent No.: US 8,696,103 B2  
(45) Date of Patent: Apr. 15, 2014

(54) TRANSFER TYPE INKJET RECORDING  
METHOD

(75) Inventors: **Shinsuke Tsuji**, Kawasaki (JP);  
**Yuichiro Kanasugi**, Tokyo (JP)

(73) Assignee: **Canon Kabushiki Kaisha**, Tokyo (JP)

(\*) Notice: Subject to any disclaimer, the term of this patent is extended or adjusted under 35 U.S.C. 154(b) by 119 days.

(21) Appl. No.: 13/298,035

(22) Filed: Nov. 16, 2011

(65) **Prior Publication Data**

US 2012/0127251 A1 May 24, 2012

(30) **Foreign Application Priority Data**

Nov. 24, 2010 (JP) ..... 2010-261603

(51) **Int. Cl.**

(51) Int. Cl.  
*B41J 2/01* (2006.01)  
(52) U.S. Cl.

(52) U.S. Cl. USPC ..... 347/103  
(58) Field of Classification Search

## Field None

See application file for complete search history

(56) **References Cited**

## U.S. PATENT DOCUMENTS

2009/0322805 A1\* 12/2009 Chiwata ..... 347/6  
2010/0079544 A1\* 4/2010 Sumi ..... 347/40

## FOREIGN PATENT DOCUMENTS

|    |             |   |   |        |       |            |
|----|-------------|---|---|--------|-------|------------|
| JP | 2001226444  | A | * | 8/2001 | ..... | C08G 18/10 |
| JP | 2003-80826  | A |   | 3/2003 |       |            |
| JP | 2003-246135 | A |   | 9/2003 |       |            |
| JP | 2008-018719 | A |   | 1/2008 |       |            |
| JP | 2009-096175 | A |   | 5/2009 |       |            |

\* cited by examiner

*Primary Examiner* — Stephen Meier

*Assistant Examiner* — Alexander C Witkowski

(74) *Attorney, Agent, or Firm* — Canon U.S.A., Inc., IP Division

## ABSTRACT

A transfer type inkjet recording method uses an aggregation liquid, in which the aggregation liquid contains a polyurethane resin having an amino group and the polyurethane resin has a number average molecular weight of 10,000 or more and 1,000,000 or lower and an amine value of 0.5 mmol/g or more and 3.0 mmol/g or lower.

**7 Claims, 1 Drawing Sheet**





TRANSFER TYPE INKJET RECORDING  
METHOD

## BACKGROUND OF THE INVENTION

## 1. Field of the Invention

The present invention relates to a transfer type inkjet recording method.

## 2. Description of the Related Art

As one of printing methods, a recording method (transfer type inkjet recording method) is mentioned which includes forming an intermediate image on an intermediate transfer body by an inkjet recording method, and transferring the intermediate image to a recording medium to form a final image. In the transfer type inkjet recording method, a method is known which includes giving an aggregation liquid which aggregates inks to an intermediate transfer body in order to increase image performance and water resistance (Japanese Patent Laid-Open No. 2003-246135). The method described in Japanese Patent Laid-Open No. 2003-246135 aggregates the inks on the intermediate transfer body with an aggregation liquid containing a cationic polymer, such as dicyandiamide resin or polyallylamine to suppress bleeding (mixture of colors of inks) to thereby increase image performance. Furthermore, by increasing the molecular weight of cationic substances, the film strength of images is increased to thereby increase the water resistance.

However, according to an examination of the present inventors, the recording method described in Japanese Patent Laid-Open No. 2003-246135 has the following problems. First, there is a problem in that the transfer properties in transferring the intermediate image on the intermediate transfer body to a recording medium are not good and the final image formed on the recording medium is distorted. This is considered to be because the aggregation properties of inks forming the intermediate image are insufficient when the printing Duty is high, so that the internal aggregation force of the intermediate image required for transferring becomes insufficient. Such a reduction in the transfer properties is particularly remarkable when a fine quality paper having relatively high surface roughness or the like is used as the recording medium.

Furthermore, there is a problem in that scratch resistances when moisture is given to printed substances which are required in commercial printed substances and the like are insufficient. The commercial printed substances are left as they are in a state where water adheres onto the printed substances, and then used after removing the water in some cases. The scratch in such a state where moisture is given thereto is referred to as "wet scratch". When the printed substances obtained by the recording method described in Japanese Patent Laid-Open No. 2003-246135 have been subjected to the wet scratch, scratch marks are generated on the images to cause considerable distortion in some cases. This is considered to occur due to the fact that when water is left on the printed substances on which images are formed, the water permeates into the printed surface so that the printed surface is swollen to be deteriorated, and then water wiping is performed in such a state, resulting in the separation of the swollen printed surface.

In the case where the inks are color inks, bleeding has sometimes occurred when high concentration images having a high printing Duty have been formed. This is considered to be because the aggregation force is not sufficient when a component which aggregates the ink is only a cationic polymer (aggregation agent), and when the ink amount is large

relative to the amount of the aggregation liquid per unit area, it becomes difficult to sufficiently aggregate the inks forming the intermediate image.

## SUMMARY OF THE INVENTION

Therefore, according to aspects the present invention provide a transfer type inkjet recording method with good transfer properties and good wet scratch resistances of the final image even when the printing Duty is high.

The above-described problems may be solved according to aspects of the following invention. More specifically, aspects of the present invention include a transfer type inkjet recording method, having an intermediate image formation process for forming an intermediate image by giving an ink containing an anionic component to an image formation surface of an intermediate transfer body to which an aggregation liquid containing an aggregation agent which aggregates the anionic component in the ink by an inkjet recording method to thereby form an intermediate image, and a transfer process for pressure-bonding a recording medium to the image formation surface on which the intermediate image is formed to transfer the intermediate image to the recording medium from the image formation surface, in which the aggregation liquid further contains a polyurethane resin having an amino group and the polyurethane resin having an amino group has a number average molecular weight of 10,000 or more and 1,000,000 or lower and an amine value of 0.5 mmol/g or more and 3.0 mmol/g or lower.

The invention can provide a transfer type inkjet recording method with good transfer properties and good wet scratch resistances of the final image even when the printing Duty is high.

Further features of the present invention will become apparent from the following description of exemplary embodiments with reference to the attached drawing.

## BRIEF DESCRIPTION OF THE DRAWING

FIGURE illustrates an example of an image recording device which performs the inkjet recording method according to aspects of the invention.

## DESCRIPTION OF THE EMBODIMENTS

Hereinafter, the invention is described in detail.

**Ink**  
The ink for use in the transfer type inkjet recording method according to aspects of the invention contains an anionic component.

Mentioned as the anionic component is one exhibiting a minus charge. Mentioned as suitable anionic components are carboxylic acid, sulfonic acid, phosphonic acid, and compounds having an anionic group in which the above-mentioned acids are neutralized by a metal salt or organic amine, and the like. The anionic component is suitably a high molecular weight substance. This is because when a component forming an ionic bond with the cationic component in the aggregation liquid is a high molecular weight substance, the film strength becomes high and the wet scratch resistances become good. The high molecular weight substance to be used as the anionic component according to aspects of the invention is suitably a dispersant which disperses color materials. When the high molecular weight substance is a dispersant which disperses color materials, the weight average molecular weight is suitably 1,000 or more and 50,000 or lower. When the high molecular weight substance is in the

shape of emulsion particles, the weight average molecular weight is suitably 1,000 or more and 10,000,000 or lower.

According to aspects of the invention, the anionic component may be a pigment having an anionic functional group or may be an anionic dye.

The ink according to aspects of the invention may contain a functional additive in order to further increase the fastness of the final image. Mentioned as the functional additive are known water soluble resin, water insoluble resin fine particles, and the like. The materials to be used are not limited insofar they can be co-exist with other ink components. The water insoluble resin fine particles refer to fine particles of a water insoluble polymer which can be dispersed in an aqueous medium by a functional group (particularly an acidic group or a salt thereof) contained therein and which does not contain a free emulsifier. Mentioned as the water insoluble polymer are, for example, water insoluble polymers and the like described in Japanese Patent Laid-Open No. 2009-096175.

The ink according to aspects of the invention may be a clear ink not containing a color material or may be a color ink containing a color material. Usable as the color material to be compounded are known dyes and pigments described in Japanese Patent Laid-Open No. 2008-018719. Moreover, in order to disperse the color material, dispersants described in Japanese Patent Laid-Open No. 2008-018719 can be used.

The ink according to aspects of the invention suitably contains water and an organic solvent. The organic solvent is suitably a water soluble material having a high boiling point and a low vapor pressure as shown below. For example, polyethylene glycol, polypropylene glycol, ethylene glycol, propylene glycol, butylene glycol, triethylene glycol, thioglycol, hexylene glycol, diethylene glycol, ethylene glycol monomethyl ether, diethylene glycol monomethyl ether, glycerin, and the like are mentioned. These substances may be used singly or in combination of two or more kinds thereof. Moreover, alcohols, such as ethyl alcohol or isopropyl alcohol, or surfactants may be added into the ink as a component for adjusting the viscosity, surface tension, and the like.

The compounding ratio of the components constituting the ink is not particularly limited and can be adjusted as appropriate in the range where ejection can be achieved in accordance with the ejection power, the diameter of a nozzle, and the like of the selected inkjet head. When the total ink amount is adjusted to 100% by mass, the color material is suitably 0.1% by mass or more and 10% by mass or lower. The organic solvent is 5% by mass or more and 40% by mass or lower. The surfactant is 0.01% by mass or more and 5% by mass or lower. Then, the balance is adjusted with water. The ink according to aspects of the invention is suitably an aqueous ink containing 40% by mass or more of water.

#### Aggregation Liquid

The aggregation liquid for use in the transfer type inkjet recording method according to aspects of the invention contains an aggregation agent and a polyurethane resin having an amino group.

It is important for the aggregation agent according to aspects of the invention to have a function of aggregating the anionic component in the ink and to be co-exist with the polyurethane resin having an amino group in the aggregation liquid. As such an aggregation agent, a metal salt which generates metal ions or an acidic compound which varies a hydrogen ion concentration (pH) is suitable. Among the above, the acidic compound is more suitable from the viewpoint of coexistence with the polyurethane resin having an amino group.

As the metal salt, one which generates the following polyvalent metal ions is used, for example. More specifically, divalent metal ions, such as  $\text{Ca}^{2+}$ ,  $\text{Cu}^{2+}$ ,  $\text{Ni}^{2+}$ ,  $\text{Mg}^{2+}$ , and  $\text{Zn}^{2+}$ , trivalent metal ions, such as  $\text{Fe}^{3+}$  and  $\text{Al}^{3+}$ , and the like are mentioned. When a liquid containing these metal salts is applied, the liquid is suitably applied as an aqueous metal salt solution. Mentioned as negative ions of metal salts are  $\text{Cl}^-$ ,  $\text{NO}_3^-$ ,  $\text{SO}_4^{2-}$ ,  $\text{I}^-$ ,  $\text{Br}^-$ ,  $\text{ClO}_3^-$ ,  $\text{RCOO}^-$  (R is a monovalent organic group), and the like.

10 The acidic compound suitably has a pH buffering ability from the viewpoint of the aggregation performance of the ink and suitably has an acid dissociation constant ( $\text{pKa}$ ) of 4.5 or lower. When the acid dissociation constant exceeds 4.5, the aggregation performance decreases, so that a complex aggregate obtained by the anionic component in the ink and the aggregation agent and a polymer compound in the aggregation liquid is difficult to sufficiently form. As an example of the acidic compound, organic carboxylic acid, organic sulfonic acid, and the like are mentioned. More specifically, 15 polyacrylic acid, acetic acid, methanesulfonic acid, glycolic acid, malonic acid, malic acid, maleic acid, ascorbic acid, succinic acid, glutaric acid, fumaric acid, citric acid, tartaric acid, lactic acid, sulfonic acid, orthophosphoric acid, pyrrolidine carboxylic acid, pyrone carboxylic acid, pyrrole carboxylic acid, furan carboxylic acid, pyridine carboxylic acid, coumarinic acid, thiophene carboxylic acid, nicotinic acid, and levulinic acid, or derivatives of these compounds, salts thereof, and the like are mentioned.

The above-described metal salts and acidic compounds 30 may be used singly or in combination of two or more kinds thereof. The content of the aggregation agent in the aggregation liquid is suitably 0.01% by mass or more and 90% by mass or lower based on the total mass of the aggregation liquid. The content thereof is more suitably 1% by mass or 35 more and still more suitably 10% by mass or more. The content thereof is more suitably 80% by mass or lower and still more suitably 70% by mass or lower. When the content thereof is lower than 0.01% by mass, the aggregation agent cannot sufficiently aggregate the anionic components in some 40 cases. When the content thereof exceeds 90% by mass, the aggregation agent is non-uniformly present as insoluble substances in the aggregation liquid depending on the type of the aggregation agent in some cases, which sometimes results in the fact that the application of the aggregation liquid or the 45 formation of the intermediate image becomes difficult.

The aggregation liquid according to aspects of the invention contains the polyurethane resin having an amino group. A feature of the polyurethane resin having an amino group (hereinafter referred to as the polyurethane resin according to 50 aspects of the invention) to be used according to aspects of the invention resides in having a high number average molecular weight and a high amine value. Specifically, the number average molecular weight is 10,000 or more and 1,000,000 or lower. The amine value is 0.5 mmol/g or more and 3.0 mmol/g or lower. The polyurethane is a polymer compound having a urethane bond ( $-\text{NHCOO}-$ ). For example, the polyurethane is obtained by reacting an isocyanate component (a compound having an isocyanate group) and a polyol component (a compound having a plurality of hydroxyl groups).

60 The number average molecular weight of the polyurethane resin according to aspects of the invention is 10,000 or more and 1,000,000 or lower. The number average molecular weight is suitably 30,000 or more, more suitably 50,000 or more, and particularly suitably 100,000 or more. The number 65 average molecular weight is suitably 900,000 or lower and more suitably 800,000 or lower. Due to the fact that the number average molecular weight is 10,000 or more, the

## 5

coating properties of the intermediate image to be obtained and the transfer properties or the scratch resistances and the wet scratch resistances of the final image are increased. In the case of the color ink, the occurrence of bleeding can be suppressed. When the number average molecular weight is 1,000,000 or lower, long-term storage stability of the aggregation liquid can be secured.

The amine value of the polyurethane resin according to aspects of the invention is 0.5 mmol/g or more and 3.0 mmol/g or lower. The amine value is suitably 0.6 mmol/g or more. The amine value is more suitably 2.5 mmol/g or lower and still more suitably 2.0 mmol/g or lower. When the amine value of the polyurethane resin according to aspects of the invention is lower than 0.5 mmol/g, it becomes difficult to sufficiently form an ionic bond of a large number of anionic components in the inks to form an aggregate, so that the coating properties of the intermediate image decrease, resulting in the fact that the transfer properties become low. In the case of color ink, bleeding occurs. Furthermore, in the final image formed on a recording medium, an excessive amount of hydrophilic anionic components deriving from the ink remains, so that the wet scratch resistances become low. When the amine value is higher than 3.0 mmol/g, an excessive amount of hydrophilic amino groups of the polyurethane resin remains relative to the anionic components particularly in the final image formed with a low Duty, so that the wet scratch resistances become low. The amine value of the polyurethane resin according to aspects of the invention is suitably 0.1 times or more and 4.5 times or lower the total acid value of the anionic components in the ink in terms of transfer properties and wet scratch resistances.

The amino group of the polyurethane resin according to aspects of the invention may be any one of a primary amine, a secondary amine, and a tertiary amine or may have a structure in which the amines are quaternized. In particular, a tertiary amine or a structure in which a tertiary amine is quaternized is suitable. In the case of a primary amine, a secondary amine, or a structure in which the amines are quaternized, the amino group has nucleophilicity. This causes a nucleophilic addition reaction in other additives contained in the aggregation liquid, so that the storage stability of the aggregation liquid decreases in some cases.

The content of the polyurethane resin according to aspects of the invention of the aggregation liquid is suitably 1% by mass or more, more suitably 5% by mass or more, and still more suitably 10% by mass or more based on the total mass of the aggregation liquid. The content thereof is suitably 90% by mass or lower, more suitably 70% by mass or lower, and still more suitably 50% by mass or lower. When the content thereof is lower than 1% by mass, the effects according to aspects of the invention are not sufficiently developed. When the content thereof exceeds 90% by mass, the addition amount of the aggregation agent becomes excessively small, so that the aggregation properties of the ink become insufficient, which sometimes results in the fact that the transfer properties of the intermediate image or the image performance of the final image decreases.

The polyurethane resin according to aspects of the invention may be in a dissolution state or may be in a dispersion state in the aggregation liquid. When the content of the polyurethane resin is large, the viscosity remarkably increases in the dissolution state. Therefore, from the viewpoint of handling properties, the dispersion state is suitable. In the case of the dispersion state, the average particle diameter (median size) of the polyurethane resin is suitably 0.01  $\mu\text{m}$  or more and 1.00  $\mu\text{m}$  or lower. When the average particle diameter is larger than 1.00  $\mu\text{m}$ , the accuracy of the ink impact position

## 6

decreases or the surface roughness of the intermediate image in transferring becomes large, which sometimes results in a reduction in the transfer properties. When the average particle diameter is smaller than 0.01  $\mu\text{m}$ , it becomes difficult to stably obtain a uniform particle diameter, which results in the fact that the particle diameter distribution increases, and thus unevenness arises in images in some cases.

When the polyurethane resin is in the dispersion state, it is suitable that the particles are coated in the final image. When the particles are not coated in the final image, light scattering occurs due to the presence of the particles particularly when the particle diameter is large, so that the glossiness of the final image decreases or water resistance decreases in some cases. Therefore, it is suitable to perform heating treatment at a temperature equal to or higher than the minimum film forming temperature of the particles in an image fixing process to sufficiently coat the particles.

According to aspects of the invention, the aggregation liquid may contain only one kind of the polyurethane resin or two or more kinds thereof.

The aggregation liquid according to aspects of the invention suitably contains water, an organic solvent, an additive, and the like. The water soluble organic solvent is suitably an organic solvent as shown below. For example, polyethylene glycol, polypropylene glycol, ethylene glycol, propylene glycol, butylene glycol, triethylene glycol, thiodiglycol, hexylene glycol, diethylene glycol, pentane diol, ethylene glycol monomethyl ether, diethylene glycol monomethyl ether, glycerin, and the like.

The pH of the aggregation liquid according to aspects of the invention is suitably 1.0 or more and 5.0 or lower from the viewpoint of the aggregation performance of the ink. The pH is more suitably 4.0 or lower and still more suitably 3.5 or lower. When the pH exceeds 5.0, the aggregation performance of the ink decreases, so that a complex aggregate obtained by the anionic component in the ink, the aggregation agent, and the polyurethane resin according to aspects of the invention is not sufficiently formed, and therefore the effects according to aspects of the invention are not sufficiently developed in some cases.

By the use of the aggregation liquid containing the polyurethane resin according to aspects of the invention, even when the printing Duty is high, the final image with good transfer properties and good wet scratch resistances can be formed. In the case of color ink, the occurrence of bleeding can be suppressed. The present inventors presume the reasons as follows. When the intermediate image is formed on the intermediate transfer body, a complex aggregation reaction occurs due to synergistic action of three components of the anionic component of the ink, the aggregation agent in the aggregation liquid, and the polyurethane resin according to aspects of the invention. Thus, sufficient aggregation performance which suppresses the occurrence of bleeding or the like can be developed independent of the ink amount. The intermediate image obtained by the complex aggregation reaction becomes an aggregate with a specifically high molecular weight and the transfer properties become very good. The image transferred to a recording medium has a specific three-dimensional crosslinking structure formed by an intermolecular hydrogen bond developed by the urethane skeleton of the polyurethane resin according to aspects of the invention and an ionic bond formed by the above-described three components, and the wet scratch resistances become good. It is considered that the film having the above-described specific three-dimensional crosslinking structure dramatically suppresses the permeation of water into the film to

thereby suppress the swelling and deterioration of the final image due to the water, so that the wet scratch resistances become good.

Transfer Type Inkjet Recording Method and Image Recording Device

Next, the transfer type inkjet recording method and the configuration of the image recording device according to aspects of the invention are described.

FIGURE is a schematic view illustrating the outline structure of an example of the image recording device according to aspects of the invention. An image recording device **1** has an intermediate transfer body **2**, an ink ejection portion **3**, an aggregation liquid supply portion **4**, a solvent removal portion **5**, and a transfer portion **6** as the main configuration and further has a cleaning portion **7** and an image fixing portion **8**. The intermediate transfer body **2** is constituted by an endless belt having a given width and has a structure in which the intermediate transfer body **2** is wound around a plurality of rollers **10**, **11**, and **12**. It is configured so that the power of a motor (not illustrated) is transmitted to at least one main roller among the plurality of rollers **10**, **11**, and **12**, and the intermediate transfer body **2** rotates by the drive of the motor outside each of the rollers **10**, **11**, and **12** in the direction indicated by the arrow A of FIGURE (hereinafter referred to as a transfer body rotation direction). Synchronizing with the rotation, the respective units of the aggregation liquid supply portion **4**, the ink ejection portion **3**, the solvent removal portion **5**, the transfer portion **6**, the cleaning portion **7**, and the image fixing portion **8** disposed therearound operate. In this embodiment, a polyurethane belt is used as a support member of the intermediate transfer body **2** in terms of strength with which the belt can bear pressurization in transferring or dimension accuracy. The support member of the intermediate transfer body **2** may be any substance insofar as the surface layer of the intermediate transfer body **2** can establish at least line contact with the recording medium **13** and is selected in accordance with the form of the image recording device to be applied or the transfer form to the recording medium **13**. For example, support members of a roller shape and a drum shape can also be suitably used.

For the intermediate transfer body **2**, properties of forming an intermediate image by the supply of ink and transferring the formed intermediate image to a recording medium to form a good final image are important. When the transfer properties are high, the ink use efficiency is good, so that the amount of the ink to be discarded is reduced and also a load of a cleaning unit is reduced. The surface of the intermediate transfer body **2** therefor is suitably an ink non-absorbing surface and more suitably an ink non-adhering surface. Furthermore, the surface suitably has elasticity for following the surface of a recording medium, such as paper, for sufficient contact. Mentioned as materials which satisfy these properties are various kinds of plastics, rubber, and the like. In particular, silicone rubber, fluorosilicone rubber, fluororubber, and the like are suitably used in terms of non-adhesiveness. The rubber sometimes has a low surface energy and poor ink receiving properties, and therefor may be surface treated in accordance with the ink to be used. Mentioned as an example of the surface treatment are chemical treatment using chemicals, physical treatment which varies the surface shape, energy irradiation treatment which emits ultraviolet

rays or plasma, and the like. According to aspects of the invention, a combination of the intermediate transfer body whose contact angle with the aggregation liquid to be used is 10° or more and 100° or lower and the aggregation liquid is extremely suitably used.

In the aggregation liquid supply portion **4**, an aggregation liquid application roll **14**, an aggregation liquid supply roll **15**, an aggregation liquid amount regulation blade **16**, and a roll coater using a facing roll **17** are disposed as units for giving the aggregation liquid onto the intermediate transfer body **2**. This forms a configuration such that the aggregation liquid which contacts the anionic component in the ink to form an aggregate is given to the surface (image formation surface) of the intermediate transfer body **2**. The aggregation liquid may be given by any one of a spray coater, squeezing, an inkjet recording method, and the like.

The aggregation liquid is applied in the aggregation liquid supply portion **4**, and thereafter the ink is given to the image formation surface of the intermediate transfer body **2** from the ink ejection portion **3** by an inkjet recording method. Thus, the intermediate image formation process is performed in which the intermediate image (mirror image) is formed on the image formation surface of the intermediate transfer body **2**. The ink ejection portion **3** is disposed at the downstream side of the transfer body rotation direction of the aggregation liquid supply portion **4**. In the ink ejection portion **3**, recording heads **18K**, **18C**, **18M**, and **18Y** corresponding to the colors of black (K), cyan (C), magenta (M), and yellow (Y) inks are provided. The respective recording heads **18K**, **18C**, **18M**, and **18Y** eject the corresponding color inks in accordance with external image signals from the ejection surface facing the intermediate transfer body **2**. Thus, the respective color inks are given to the image formation surface of the intermediate transfer body **2**. For the ink ejection portion **3**, a continuous system and also one which ejects ink by an on-demand system using an electric heat conversion element (heat generation element), an electromechanical conversion element (piezoelectric element), or the like can also be used. As the form of the ink ejection portion **3**, with respect to the configuration of FIGURE, for example, a line head type recording head obtained by arranging ink ejection ports in the direction orthogonal to the drawing can be used. Moreover, one may be acceptable which performs recording using a recording head in which ejection ports are arranged along the tangent of the intermediate transfer body **2** or in a given range of the circumferential direction and scanning the same in the axial direction. Furthermore, a recording head can also be used corresponding to the number of colors of inks for use in the image formation.

The solvent removal portion **5** is provided with a drying furnace **19** having a heating fan (not illustrated) in order to remove a liquid component from the intermediate image formed on the image formation surface of the intermediate transfer body **2** to a degree where good transfer can be achieved. When a reduction in the liquid component is insufficient, a surplus liquid overflows to distort the image in the transfer process which is the following process or the transfer properties decrease in some cases. Various measures which have been used heretofore can all be suitably applied as a measure for reducing the liquid component. Specifically, a measure using evaporation by heating, a measure for blowing

dry air, a liquid absorption measure by an absorber, a measure containing a combination thereof, or the like can be suitably used.

Next, a transfer process is performed which includes pressure-bonding a recording medium **13** to the image formation surface on which the intermediate image is formed to transfer the intermediate image from the image formation surface to the recording medium **13**. In the device illustrated in FIGURE, the intermediate transfer body **2** and the recording medium **13** are pressurized in such a manner as to be sandwiched by the roller **11** and the pressurization roller **20** to thereby realize efficient image transfer. According to this aspect, the liquid component in the ink already decreases on the intermediate transfer body **2** in this stage and the viscosity of the ink is increased, and therefore a good final image can be formed even using a recording medium with low ink absorbency, such as a coated paper.

In a conveyance portion **8**, the recording medium **13** is conveyed from a paper feed tray **21** to a paper discharge tray **22** passing through the transfer portion **6**. For the conveyance mechanism of a cut sheet, one using a roller and a guide is used, for example. In order to suppress the occurrence of double feed or the like of the recording media **13** to perform safe conveyance, a mechanism for blowing air from the side surface of the recording medium loaded on the tray to facilitate the conveyance of the recording medium **13** may be used. In order to protect the recording medium **13** from expanding and contracting due to changes in humidity, a temperature control mechanism may be used. As the shape of the recording medium **13**, a cut sheet is used in this embodiment but a roll-shaped continuous sheet may be acceptable.

The image fixing portion **8** is disposed at the recording medium discharging side of the transfer portion **6** (right side of FIGURE). In the image fixing portion **8**, two fixing rollers **35** and **36** are provided on the front and back surfaces of the recording medium **13**. By pressurizing and heating the image transferred to be formed on the recording medium **13** by these fixing rollers **35** and **36**, the fixability of the recorded image

carbon black MCF88 to oxidation reaction treatment using known hypochlorous acid and is an anionic component.

TABLE 1

| Color material | Name                                                                              |
|----------------|-----------------------------------------------------------------------------------|
| 1              | Carbon black: MCF88 (manufactured by Mitsubishi Chemical Corporation)             |
| 2              | Pigment Blue 15 (manufactured by Dainichiseika Color & Chemicals Mfg. Co., Ltd)   |
| 3              | Pigment Red 7 (manufactured by Dainichiseika Color & Chemicals Mfg. Co., Ltd)     |
| 4              | Pigment Yellow 74 (manufactured by Dainichiseika Color & Chemicals Mfg. Co., Ltd) |
| 5              | Oxide body of carbon black MCF88 (Acid value 0.8 mmol/g)                          |

As a water soluble resin (dispersant), a neutralization salt (Weight average molecular weight: 8700, Acid value: 3.9 mmol/g, Anionic component) obtained by a potassium hydrate of a styrene-methacrylic acid-benzyl acrylate copolymer was used. The water soluble resin was obtained by polymerizing by the method described in Japanese Patent Laid-Open No. 2009-096175.

A batch type vertical sand mill (manufactured by IMEX) was filled with each color material and a dispersant, glass beads having a diameter of 1 mm were charged therein as a medium, water-cooling was performed, and dispersion treatment was performed for 3 hours. The obtained dispersion liquid was placed on a centrifugal separator to remove coarse particles, thereby producing inks having color materials with a weight average particle diameter of 100 to 200 nm with the composition shown in Table 2. The total acid value was measured using a potential difference automatic titrator (AT-510, manufactured by Kyoto Electronics Manufacturing Co., Ltd.).

TABLE 2

| Color material | Dispersant |               |      |               | Surfactant      |                            |              |                       |                           |
|----------------|------------|---------------|------|---------------|-----------------|----------------------------|--------------|-----------------------|---------------------------|
|                | Type       | Amount <part> | Type | Amount <part> | Glycerin <part> | Polyethylene glycol <part> | Water <part> | (AcetylenolEH) <part> | Total acid value <mmol/g> |
| Black ink 1    | 1          | 2             | 1    | 2             | 10              | 5                          | 80           | 1                     | 3.6                       |
| Cyan ink 1     | 2          | 2             | 1    | 2             | 10              | 5                          | 80           | 1                     | 3.6                       |
| Yellow ink 1   | 3          | 2             | 1    | 2             | 10              | 5                          | 80           | 1                     | 3.6                       |
| Magenta ink 1  | 4          | 2             | 1    | 2             | 10              | 5                          | 80           | 1                     | 3.6                       |
| Black ink 2    | 5          | 2             | —    | —             | 10              | 5                          | 80           | 1                     | 0.7                       |

on the recording medium **13** can be increased. As the fixing rollers **35** and **36**, a pair of rollers containing one pressurization roller and one heating roller is suitable.

## EXAMPLES

Hereinafter, Examples and Comparative Examples according to aspects of the invention are described below but the invention is not limited thereto. In the following description, "part" and "parts" are all based on mass.

Ink

As color materials, pigments shown in Table 1 were used. A color material **5** is an oxide body obtained by subjecting

## Aggregation Liquid

First, polymer compounds shown in Table 3 were synthesized. Polymer compounds 1 to 3 and comparative polymer compounds 1 and 2 were obtained by synthesizing monomer species shown in Table 3 by the same technique as that of Japanese Patent Laid-Open No. 2003-80826. The number average molecular weight was measured using a gel permeation chromatograph (RID-10A, manufactured by Shimadzu Corp.). The amine value was calculated from the structure of the monomer species. The average particle diameter was measured using a particle diameter distribution meter (Nano track UPA-EX150 manufactured by Nikkiso).

TABLE 3

|                                | Monomer species or Polymer compound                                                                                                                                                                                                                    | Charging ratio<br><part> | Number average<br>molecular weight | Amine value<br><mmol/g> | Average particle<br>diameter (Median<br>diameter) <μm> |
|--------------------------------|--------------------------------------------------------------------------------------------------------------------------------------------------------------------------------------------------------------------------------------------------------|--------------------------|------------------------------------|-------------------------|--------------------------------------------------------|
| Polymer compound 1             | Polyester diol (TA-22-419A, manufactured by Hitachi Chemical Co., Ltd.)<br>Trimethylol propane<br>N-methyl-N,N-diethanol amine<br>Isophorone diisocyanate                                                                                              | 240<br>10<br>200<br>200  | 720,000                            | 2.9                     | 0.03                                                   |
| Polymer compound 2             | Polycarbonate diol (Nippollan981, manufactured by Nippon Polyurethane Industry Co., Ltd.)<br>Polyethylene glycol PEG600s<br>(manufactured by Daiichi Kogyo Seiyaku Co., Ltd.)<br>N-methyl-N,N-diethanol amine<br>4,4'-dicyclohexylmethane diisocyanate | 250<br>10<br>32<br>200   | 450,000                            | 0.6                     | 0.02                                                   |
| Polymer compound 3             | Polybutylene adipate diol<br>Trimethylol propane<br>N-methyl-N,N-diethanol amine<br>Isophorone diisocyanate                                                                                                                                            | 300<br>10<br>50<br>200   | 50,000                             | 0.9                     | 0.05                                                   |
| Comparative polymer compound 1 | Polyester diol (TA-22-419A, manufactured by Hitachi Chemical Co., Ltd.)<br>Trimethylol propane<br>N-methyl-N,N-diethanol amine<br>Isophorone diisocyanate                                                                                              | 240<br>10<br>40<br>200   | 8,000                              | 0.8                     | 0.04                                                   |
| Comparative polymer compound 2 | Polybutylene adipate diol<br>N-methyl-N,N-diethanol amine<br>Isophorone diisocyanate                                                                                                                                                                   | 300<br>10<br>200         | 420,000                            | 0.2                     | 0.03                                                   |
| Comparative polymer compound 3 | Dicyan diamide•diethylene triamine condensate<br>(Trade name: UnisenseKHP10P, manufactured by Senka Corporation, Solid content 100%)                                                                                                                   | —                        | —                                  | —                       | —                                                      |
| Comparative polymer compound 4 | Polyallylamine hydrochloride<br>(Trade name: PAA-HCL-05, manufactured by Nitto Boseki Co., Ltd., Solid content 40%)                                                                                                                                    | —                        | —                                  | —                       | —                                                      |

Each polymer compound was identified using a <sup>1</sup>H-NMR spectral method (Used device; Avance 500 (Trade name), manufactured by Bruker), a <sup>13</sup>C-NMR spectral method (Used device; Avance 500 (Trade name), manufactured by Bruker), and an infrared spectroscopy (Used device; Spectrum One (Trade name), manufactured by PerkinElmer). As a result, it was confirmed that each of the polymer compounds 1 to 3 and the comparative polymer compounds 1 and 2 was the polyurethane resin having an amino group. In contrast, it was confirmed that each of the comparative polymer compounds 3 and 4 was not the polyurethane resin.

The aggregation liquids shown in Table 4 were produced using the above-described polymer compounds. The pKa of glutaric acid of Table 4 is 4.13 and the pKa of levulinic acid of Table 4 is 4.44.

#### Recording Method

Printed substances on which the final image was formed were obtained using the above-described inks and aggregation liquids by the following transfer type inkjet recording method.

#### (A) Aggregation Liquid Supply Process

A material was prepared in which the surface of a 0.4 mm PET film was coated with a silicone rubber (Trade name; KE12, manufactured by Shin-Etsu Chemicals Co., Ltd.) having a rubber hardness of 40° with a thickness of 0.3 mm. The material was subjected to surface hydrophilization using a parallel flat plate type atmospheric pressure plasma treatment device (APT-203, manufactured by Sekisui Chemical) to form the intermediate transfer body to be used in this Example. The aggregation liquid was given to the intermediate transfer body in a liquid state using a roll coater with a coating amount of 5.0 g/m<sup>2</sup>.

TABLE 4

| Type                             | Polymer compound               | Aggregation agent |                 | Organic solvent  |                 |                  |
|----------------------------------|--------------------------------|-------------------|-----------------|------------------|-----------------|------------------|
|                                  |                                | Amount<br><part>  | Type            | Amount<br><part> | Type            | Amount<br><part> |
| Aggregation liquid 1             | Polymer compound 1             | 20                | Glutaric acid   | 35               | 1,5-pentanediol | 10               |
| Aggregation liquid 2             | Polymer compound 2             | 20                | Glutaric acid   | 35               | 1,5-pentanediol | 10               |
| Aggregation liquid 3             | Polymer compound 3             | 20                | Glutaric acid   | 35               | 1,5-pentanediol | 10               |
| Aggregation liquid 4             | Polymer compound 2             | 20                | Calcium nitrate | 35               | 1,5-pentanediol | 10               |
| Aggregation liquid 5             | Polymer compound 1             | 20                | Levulinic acid  | 35               | 1,5-pentanediol | 10               |
| Comparative aggregation liquid 1 | Comparative polymer compound 1 | 20                | Glutaric acid   | 35               | 1,5-pentanediol | 10               |
| Comparative aggregation liquid 2 | Comparative polymer compound 2 | 20                | Glutaric acid   | 35               | 1,5-pentanediol | 10               |
| Comparative aggregation liquid 3 | Comparative polymer compound 3 | 10                | —               | —                | 1,5-pentanediol | 10               |
| Comparative aggregation liquid 4 | Comparative polymer compound 4 | 65                | —               | —                | 1,5-pentanediol | 10               |
| Comparative aggregation liquid 5 | —                              | —                 | Glutaric acid   | 35               | 1,5-pentanediol | 10               |

## (B) Intermediate Image Formation Process

The ink was given to the image formation surface of the intermediate transfer body to which the aggregation liquid was given by an inkjet device (Nozzle arrangement density 1200 dpi, Ejection amount 4  $\mu$ l) to thereby form an intermediate image.

## (C) Transfer Process

A recording medium (Fine quality paper, Trade name; OK prince high quality EH, manufactured by Oji Paper Co., Ltd.) was pressure-bonded to the image formation surface of the intermediate transfer body with a pressurization roller to transfer the intermediate image to the recording medium.

## (D) Fixing Process

The recording medium to which the intermediate image was transferred was heated for 2 minutes with 100° C. hot wind to fix the image. Thus, a recording medium on which the final image was formed was obtained.

The ink and the aggregation liquid used in each Example are shown in Table 5. The "Amine value/Acid value" in Table 5 is a ratio of the amine value of the polyurethane resin contained the aggregation liquid relative to the total acid value of the anionic component in the ink.

TABLE 5

|             | Ink         | Aggregation liquid               | Amine value/Acid value |
|-------------|-------------|----------------------------------|------------------------|
| Example 1   | Black ink 1 | Aggregation liquid 1             | 0.8                    |
| Example 2   | Black ink 1 | Aggregation liquid 2             | 0.2                    |
| Example 3   | Black ink 1 | Aggregation liquid 3             | 0.2                    |
| Example 4   | Black ink 1 | Aggregation liquid 4             | 0.2                    |
| Example 5   | Black ink 2 | Aggregation liquid 1             | 4.1                    |
| Example 6   | Black ink 1 | Aggregation liquid 5             | 0.8                    |
| Comparative | Black ink 1 | Comparative aggregation liquid 1 | 0.2                    |
| Example 1   | Comparative | Black ink 1                      | 0.1                    |
| Comparative | Black ink 1 | Comparative aggregation liquid 2 | —                      |
| Example 2   | Black ink 1 | Comparative aggregation liquid 3 | —                      |
| Comparative | Black ink 1 | Comparative aggregation liquid 4 | —                      |
| Example 4   | Black ink 2 | Comparative aggregation liquid 5 | —                      |
| Comparative | Black ink 1 | —                                | —                      |
| Example 6   | Black ink 1 | —                                | —                      |

## Evaluation

In the intermediate image formation process in the above-described recording method, 2 cm×2 cm intermediate images were formed on the intermediate transfer body with a recording density of 10% Duty, 100% Duty, and 350% Duty. The transfer properties to the recording medium, wet scratch resistances, and bleeding of the obtained intermediate images were evaluated based on the following criteria.

## Transfer Properties

The intermediate transfer bodies after the transfer process were observed under an optical microscope to evaluate an ink remaining area ratio of each intermediate image based on the following criteria. The remaining area ratio was calculated by subjecting the image data obtained by the optical microscope to image processing. The case where all the inks transfer to the recording medium and the intermediate image does not remain refers to a state where the remaining area ratio is 0%.

A: The ink remaining area ratio on the intermediate transfer body is 0% or more and lower than 5%.

B: The ink remaining area ratio on the intermediate transfer body is 5% or more and lower than 10%.

C: The ink remaining area ratio on the intermediate transfer body is 10% or more and lower than 20%.

D: The ink remaining area ratio on the intermediate transfer body is 20% or more and lower than 30%.

E: The ink remaining area ratio on the intermediate transfer body is 30% or more.

## 5 Wet Scratch Resistances

The final images (2 cm×2 cm) obtained by transferring the 2 cm×2 cm intermediate images to the recording medium were evaluated for the wet scratch resistances. First, the O.D. (Optical density) of the formed final image was measured.

10 Next, 0.2 ml of water droplets was added dropwise onto the final images, and the final images were allowed to stand for 3 minutes. Thereafter, scratch wiping (wet scratch) was performed with a cleaning paper, and the O.D. of the center of the portion where the water droplets were added dropwise was measured. From these measurement results, the O.D. maintaining ratio was evaluated based on the following criteria. "O.D. maintaining ratio=100×(O.D. after wet scratch)/(O.D. before wet scratch)" was established. The "O.D." was measured using a spectrophotometer (Trade name; Spectrolino manufactured by Gretag Macbeth AG).

15 A: The O.D. maintaining ratio is 99% or more.

B: The O.D. maintaining ratio is 95% or more and lower than 99%.

C: The O.D. maintaining ratio is 90% or more and lower than 95%.

20 D: The O.D. maintaining ratio is 80% or more and lower than 90%.

E: The O.D. maintaining ratio is 60% or more and lower than 80%.

## Bleeding

25 The aggregation liquid was given to the entire surface of the intermediate transfer body by the above-described recording method, and thereafter a square 2 cm on a side (100% Duty) was formed with the black ink 1. Immediately after the formation thereof, squares 2 cm on a side (100% Duty) were

30 formed with the cyan ink 1, the yellow ink 1, and the magenta ink 1 in such a manner as to be adjacent to the three sides of the square formed with the black ink 1. Similarly as above, patterns were also formed in which four squares with 10% Duty and four squares with 350% Duty were formed. Next, the boundary portion of the intermediate images on the intermediate transfer body was observed under an optical microscope. The boundary portions refer to the boundary portion of the square formed with the black ink 1 and the square formed with the cyan ink 1, the boundary portion of the square formed with the black ink 1 and the square formed with the yellow ink

35 1, and the boundary portion of the square formed with the black ink 1 and the square formed with the magenta ink 1. Then, among the bleeding occurring in each boundary portion, the portion where the bleeding level was the highest was calculated by image processing for the area ratio of the bleeding portion relative to the area of one square, and evaluated based on the following criteria.

40 A: The bleeding area ratio is lower than 0.1%. B: The bleeding area ratio is 0.1% or more and lower than 1.0%.

C: The bleeding area ratio is 1.0% or more and lower than 10.0%.

45 D: The bleeding area ratio is 10.0% or more.

The above evaluation results are shown in Table 6.

TABLE 6

| 60<br>Printing Duty | Transfer properties |    |     | Wet scratch resistances |    |     | Bleeding |    |     |
|---------------------|---------------------|----|-----|-------------------------|----|-----|----------|----|-----|
|                     | <% Duty>            | 10 | 100 | 350                     | 10 | 100 | 350      | 10 | 100 |
| Example 1           | A                   | A  | A   | B                       | A  | A   | A        | A  | A   |
| Example 2           | A                   | A  | A   | B                       | A  | A   | A        | A  | A   |
| Example 3           | A                   | A  | B   | B                       | B  | B   | A        | A  | A   |

## 15

TABLE 6-continued

| Printing Duty | Transfer properties |     |     | Wet scratch resistances |     |     | Bleeding |     |     | 5  |
|---------------|---------------------|-----|-----|-------------------------|-----|-----|----------|-----|-----|----|
|               | 10                  | 100 | 350 | 10                      | 100 | 350 | 10       | 100 | 350 |    |
| <% Duty>      |                     |     |     |                         |     |     |          |     |     |    |
| Example 4     | A                   | A   | A   | B                       | A   | B   | A        | A   | A   |    |
| Example 5     | A                   | A   | B   | B                       | B   | B   | B        | B   | B   |    |
| Example 6     | A                   | A   | A   | B                       | A   | A   | A        | A   | A   |    |
| Comparative   | B                   | B   | C   | C                       | C   | D   | B        | B   | C   | 10 |
| Example 1     |                     |     |     |                         |     |     |          |     |     |    |
| Comparative   | B                   | B   | C   | C                       | C   | D   | B        | C   | C   |    |
| Example 2     |                     |     |     |                         |     |     |          |     |     |    |
| Comparative   | C                   | C   | D   | D                       | C   | D   | C        | C   | D   | 15 |
| Example 3     |                     |     |     |                         |     |     |          |     |     |    |
| Comparative   | C                   | C   | D   | D                       | C   | E   | C        | C   | D   |    |
| Example 4     |                     |     |     |                         |     |     |          |     |     |    |
| Comparative   | C                   | C   | D   | E                       | E   | E   | C        | C   | D   |    |
| Example 5     |                     |     |     |                         |     |     |          |     |     |    |
| Comparative   | E                   | E   | E   | E                       | E   | E   | C        | D   | D   |    |
| Example 6     |                     |     |     |                         |     |     |          |     |     |    |

The transfer type inkjet recording methods of Examples 1 to 6 are excellent in all of the transfer properties, wet scratch resistances, and bleeding.

In contrast, the transfer type inkjet recording method of Comparative Example 1 in which the number average molecular weight of the polyurethane resin was lower than 10,000 was not excellent in the transfer properties, wet scratch resistances, and bleeding. The transfer type inkjet recording method of Comparative Example 2 in which the amine value of the polyurethane resin is lower than 0.5 mmol/g was not excellent in the transfer properties, wet scratch resistances, and bleeding. The transfer type inkjet recording methods of Comparative Examples 3, 4, and 5 in which the aggregation liquid does not contain the polyurethane resin were not excellent in the transfer properties, wet scratch resistances, and bleeding. The transfer type inkjet recording method of Comparative Example 6 which does not use the aggregation liquid was not excellent in the transfer properties, wet scratch resistances, and bleeding.

While the present invention has been described with reference to exemplary embodiments, it is to be understood that the invention is not limited to the disclosed exemplary embodiments. The scope of the following claims is to be accorded the broadest interpretation so as to encompass all such modifications and equivalent structures and functions.

This application claims the benefit of Japanese Patent Application No. 2010-261603 filed Nov. 24, 2010, which is hereby incorporated by reference herein in its entirety.

## 16

What is claimed is:

1. A transfer type inkjet recording method, comprising: an aggregation liquid applying process for applying an aggregation liquid containing an aggregation agent to an image formation surface of an intermediate transfer body;

an intermediate image formation process for forming an intermediate image by giving by an inkjet recording method an ink containing an anionic component which aggregates by reacting with the aggregation agent to the image formation surface of the intermediate transfer body on which the aggregation liquid is already applied to thereby form an intermediate image; and

a transfer process for pressure-bonding a recording medium to the image formation surface on which the intermediate image is formed to transfer the intermediate image to the recording medium from the image formation surface,

wherein the aggregation liquid further contains a polyurethane resin having an amino group;

wherein a number average molecular weight of the polyurethane resin is 10,000 or more and 1,000,000 or less; and

wherein an amine value of the polyurethane resin is 0.5 mmol/g or more and 3.0 mmol/g or less.

2. The transfer type inkjet recording method according to claim 1, wherein a ration of the amine value of the polyurethane resin relative to the total acid value of the anionic component in the ink is 0.1 or more and 4.5 or less.

3. The transfer type inkjet recording method according to claim 2, wherein the total acid value of the anionic component in the ink is obtained by measuring an ink by use of a potential difference automatic titrator.

4. The transfer type inkjet recording method according to claim 1, wherein the ink contains a dispersant.

5. The transfer type inkjet recording method according to claim 1, wherein the aggregation agent is a metal salt or an acidic compound.

6. The transfer type inkjet recording method according to claim 5, wherein the aggregation agent is an acidic compound.

7. The transfer type inkjet recording method according to claim 1, wherein the number average molecular weight of the polyurethane resin is 100,000 or more and 800,000 or less.

\* \* \* \* \*